

April 13, 1943.

J. W. STALLINGS

2,316,746

FLOOR AND WALL COVERING

Filed July 24, 1941



FIG. 2.



FIG. 1.

INVENTOR

WITNESS:

Robt. P. Kitchel.

James William Stallings  
BY  
John F. Bergin  
ATTORNEY.

## UNITED STATES PATENT OFFICE

2,316,746

## FLOOR AND WALL COVERING

James William Stallings, Haddon Heights, N. J.,  
assignor to Rohm & Haas Company, Philadelphia, Pa., a corporation of Delaware

Application July 24, 1941, Serial No. 403,833

6 Claims.

(Cl. 154—25)

This invention relates to non-buckling, non-distorting linoleum for floor and wall coverings, having a woven cotton backing or support.

Although burlap backing has been satisfactory for heavy floor coverings, it has not been so for thinner linoleum, particularly that used for wall coverings, as the coarse nature of the burlap cloth imparts a fabric-like effect on the wearing surface of the linoleum. Recently cotton fabrics have been used experimentally to replace burlap, but this substitution has not provided a satisfactory product. This replacement is particularly important at the present time because of difficulties encountered in obtaining burlap and of the desire to use domestic supplies of cotton.

The linoleum heretofore prepared with a cotton backing has not been fully satisfactory, because under the influence of water or moisture curling and buckling have occurred. Floor or wall coverings of this type, even though held with a waterproof cement, frequently open at the seams.

It is an object of this invention to prepare linoleum floor or wall covering which is not distorted by moisture or water and which remains smooth and plane when applied to a surface.

It has now been found that non-buckling, distortion-free linoleum may be prepared by impregnating a cotton cloth with a solution of a water-soluble carbamide-formaldehyde condensate to impart thereto about 10% to about 20% of resin, referred to the weight of the cloth, drying the cloth, applying to one face thereof a linoleum coating composition, and curing the coating on the cloth. If desired, preliminary to the application of the coating composition there may be applied to the dry cloth a sealing coat of a thick pigmented lacquer or "dope." This improves the adhesion of the linoleum materials to the base.

Figure 1 of the drawing is a cross sectional view of the floor and wall covering of this invention. Figure 2 is a perspective view of same.

As a suitable water-soluble carbamide-formaldehyde condensate there may be used the soluble methylol carbamides prepared from urea, thiourea, melamine, or the like, or from mixtures of such carbamides. There may also be used the water-soluble reaction products of a carbamide, formaldehyde, and a water-soluble alcohol such as methanol, ethanol, ethylene glycol, or glycerol, which reaction products are included within the term "water-soluble car-

bamide - formaldehyde condensate." Aqueous solutions containing 8% to 30% of such a condensate may be used for impregnating the cotton cloth. Excess solution is removed by squeezing, slot-extracting, or other suitable procedure. The amount of condensate retained by the fabric depends upon the concentration of the solution used and upon the extent of removal of solution.

10 To the impregnating solution there is preferably added an acid-type catalyst for hardening the condensate. There may be used as a catalyst a weak acid, such as acetic, formic, or lactic acid, an acid salt, such as mono- or di-methylamine hydrochloride, or an ammonium salt, such as ammonium phosphate or ammonium thiocyanate. These catalysts are used at concentrations which do not cause coagulation or gelation of the treating solution. The addition of ammonia to this solution helps to prevent premature coagulation during application of the solution to the fabric.

There may also be used in the impregnating solution a wetting and penetrating agent, such as sodium octylphenoxyethyl sulfate or sodium octylphenoxyethoxyethoxyethyl sulfonate. The use of a wetting agent is of particular value when grey goods or sized cotton fabrics are used for backing.

30 After the cotton cloth has been impregnated with a solution containing a urea-formaldehyde or other carbamide-formaldehyde condensate, it is dried on cans or in an enclosed drier at normal or elevated temperature. At this point it is usually desirable, if the cloth has not already been sized, to increase the body and weight of the cloth by sizing with a starchy composition. The desirability of this operation will depend on the construction and weight of the cloth, upon the amount of size already present, and upon the nature of the coating materials to be applied thereto. When the construction is open and of light weight, sizing becomes particularly desirable.

45 As the coating or overlay there may be used the usual linoleum mix based on linoxyn. This may be calendered or pressed onto the prepared base which is substantially dry and hard. If desired, the composite sheet may be embossed.

50 After the fabricated sheet has been cured by stoving in the usual manner, there results a covering material which rolls well and yet may be spread evenly and easily on floor or wall. Since it is not sensitive to moisture, it remains 55 flat and smooth without curling or buckling.

As typical of the preparation of covering material, the following examples are cited.

*Example 1*

A 67 x 40, 2 yd. grey cotton sheeting was padded through a solution containing 15% of water-soluble methylol urea, 0.3% of ammonium thiocyanate, and 0.4% of sodium isoctylphenoxyethoxyethyl sulfonate. The cloth was then dried on cans and passed through a size bath prepared from 100 lbs. of converted corn starch 10 lbs. of talc, 20 lbs. of glue, and 1000 lbs. of water, and again dried on a stack of cans heated with steam at 10 lbs. pressure. The sized fabric was then coated with a pigmented lacquer paste prepared from 27 parts of microcellulose, 53 parts of castor oil, 20 parts of titanium oxide, and 200 parts of solvent consisting of 35% of ethanol, 25% of ethyl acetate, 5% of butyl acetate, and 25% of toluol. The lacquer coat was dried by passing the cloth through a steam-heated oven. There was then calendered onto the coated fabric a linoxyn mix made from 10 parts of linoxyn and 17 parts of fillers and pigments. The sheet was stoved for four days at 190-200° F. The product resisted buckling and curling when moistened or steamed.

*Example 2*

Another lot of cotton sheeting in the grey with the warp heavily sized was padded through a solution containing 10% of a water-soluble condensate of urea, formaldehyde, and a small amount of thiourea, 0.1% of ammonium phosphate, 0.1% of sodium sulfate, and 0.5% of sodium isoctylphenoxyethyl sulfate. The cloth was then passed over cans heated to 300° F. The dry cloth was then sized as in the previous example, coated with a lacquer "dope," calendered with a linoleum mix, and stoved. The finished product was entirely satisfactory as a wall covering, having a smooth, plane surface and remaining flat when wet.

*Example 3*

A piece of 62 x 48, 1.9 yd. cotton sheeting was padded through a solution containing 9% of methylol urea, 0.75% of the water-soluble wetting agent prepared by reaction of octylphenol and ethylene oxide, and 10% of an emulsion containing 32% of a non-drying oil-modified alkyd resin, 8% of an organic solvent-soluble condensate of urea, formaldehyde, and butanol, and 3% of cetyltrimethylammonium acetate as an emulsifier. The cloth was dried and heated for 12 minutes in a tenter at 300° F. The cloth was then sized, dried, coated with a lacquer "dope," dried again, calendered with a thin layer of linoleum mix, and stoved, as in the

above examples. The wall covering thus obtained remained flat when wet and was entirely satisfactory in all respects.

In the processing of cotton cloth with a carbamide-formaldehyde condensate results comparable to those obtained in the above examples are obtained by impregnating cloth coated with a linoleum mix and then stoving or heating the floor or wall covering. This method, however, is somewhat less uniform in results than that of the examples.

During the processing of the backing, tension is necessarily applied to the cloth. The amount of tension is desirably of the same order as is encountered when the coated cloth is festooned during stoving.

I claim:

1. The process of preparing a non-buckling, distortion-free linoleum having a woven cotton back which comprises impregnating cotton cloth with a solution of a water-soluble carbamide-formaldehyde condensate to impart about 10% to about 20% of condensate to the cloth, drying the cloth, applying a linoleum coating composition to one face of the cloth, and heating the coated cloth.
2. The process of claim 1 in which the carbamide-formaldehyde condensate is one obtained from urea and formaldehyde.
3. The process of preparing non-buckling, distortion-free linoleum and wall covering having a cotton back which comprises impregnating cotton cloth with a water-soluble carbamide-formaldehyde condensate to impart about 10% to about 20% of condensate to the cloth, drying the cloth, sizing the cloth, applying to one face thereof a layer of a linoleum coating composition, and heating the coated cloth.
4. The process of preparing non-buckling, distortion-free linoleum and wall covering having a cotton back which comprises impregnating cotton cloth with about 10% to about 20% of a urea-formaldehyde condensate based on the weight of the cloth, drying the impregnated cloth, coating the dried cloth with a lacquer, applying to the lacquered face thereof a layer of a linoleum coating composition, and heating the coated cloth.
5. A distortion-free, non-buckling wall and floor covering comprising a cotton backing containing about 10% to about 20% of a carbamide-formaldehyde resin and a linoleum mix overlay.
6. A distortion-free non-buckling wall and floor covering comprising a cotton backing containing about 10% to about 20% of a urea-formaldehyde resin and a linoleum mix overlay.

JAMES WILLIAM STALLINGS.